

May 11, 1937.

F. L. WHITE

2,080,019

HARDENING PHOTOGRAPHIC EMULSION

Filed Sept. 10, 1936

*Fig.1.*



*Fig.2.*



*Fig.3.*



*Frank L. White,*  
INVENTOR:

BY

*Newton M. Penruis*  
*R. Frank Smith*  
ATTORNEYS.

## UNITED STATES PATENT OFFICE

2,080,019

## HARDENING PHOTOGRAPHIC EMULSION

Frank L. White, Rochester, N. Y., assignor to  
Eastman Kodak Company, Rochester, N. Y., a  
corporation of New Jersey

Application September 10, 1936, Serial No. 100,137

15 Claims. (Cl. 95—7)

This invention relates to hardening agents for photographic gelatin and emulsions, and to a method for hardening such gelatin and emulsions.

5 A number of agents for hardening photographic gelatin or emulsions have been suggested in the literature. These include dialdehydes and bromine derivatives of monoaldehydes, such as dibromocrolein. Some of the hardening agents 10 previously suggested have a tendency to fog a sensitive photographic emulsion, and in determining the utility of the various hardening agents, the melting point of the gelatin is ordinarily taken as the criterion of the hardening 15 action produced.

I have found that the halogen-substituted aldehyde acids are useful for hardening photographic gelatin and emulsions. These compounds do not fog a photographic emulsion, and permit processing of the emulsion at elevated temperatures. I have not relied upon the melting point produced 20 by addition of my hardening agents to the emulsion, but have tested them by carrying out the photographic processes including developing, 25 rinsing, fixing and washing at high temperatures to determine the ability of the hardening emulsion to withstand processing at these high temperatures, since this test is obviously more significant.

30 In the accompanying drawing, Fig. 1 is an enlarged sectional view of a film having a hardened emulsion made according to my invention, Fig. 2 is an enlarged sectional view of a film having a hardened inter-layer and a hardened 35 filter layer, and Fig. 3 is an enlarged sectional view of a film having a hardened anti-halation backing layer.

In the practice of my invention, the compounds used are incorporated in the gelatin or emulsion 40 by dissolving them in a suitable solvent which does not adversely affect the sensitive photographic emulsion, and mixing the solution of the hardening agent with the gelatin or emulsion. The compounds which I use for hardening 45 gelatin comprise the halogen-substituted aldehyde acids, such as mucobromic and mucochloric acids. The formulae for these compounds are as follows:

50 Mucobromic acid:



Mucochloric acid:



These compounds may be produced according 60 to the procedure of Simonis, Berichteder Deut-

schen Chemischen Gesellschaft, vol. 32, (1899), page 2084.

The following examples illustrate methods of incorporating the hardening agents in photographic emulsions according to my invention. 5

## Example I

To about 10 cc. of ethyl alcohol there was added 0.05 gram of mucobromic acid to form a solution of the acid in alcohol. This solution 10 was added to 225 grams (about 215 cc.) of a high speed, high contrast photographic emulsion (containing about 7% gelatin). After mixing the solution of the hardening agent with the emulsion, the mixture was immediately coated 15 on a suitable support, such as a transparent cellulose acetate support, and permitted to dry. A similar emulsion to which no hardening agent had been added was also coated on a support and permitted to dry in a similar manner. These 20 emulsions were then exposed and subjected to development, rinsing, fixing and washing at 85° F. Observation of the resulting plates showed that the emulsion to which the mucobromic acid had been added had a very definite increase in hard- 25 ening over the control, and was not fogged.

## Example II

To about 10 cc. of ethyl alcohol there was added 0.1 gram of mucochloric acid to form a 30 solution of the acid in alcohol. This solution was added to 225 grams of a high speed, high contrast photographic emulsion (containing about 7% gelatin), and after mixing the solution of the hardening agent with the emulsion, the 35 emulsion was coated on a transparent cellulose acetate support. A similar emulsion to which no hardening agent had been added was coated on a support, and the two emulsions were exposed and processed including development, rinsing, fixing and washing at both 30° F. and 100° F. The emulsion to which no hardening agent had been 40 added was quite soft at 85° F. and started to melt during development at 100° F. The emulsion to which the hardening agent had been 45 added withstood processing at 85° F. quite satisfactorily, and although it was somewhat soft when processed at 100° F., it did not melt as did the control sample.

## Example III

To about 25 cc. of ethyl alcohol there was added 0.4 g. of mucochloric acid to form a solution of the acid in alcohol. This solution was added to 250 g. of a gelatin solution consisting of 7 percent 55 gelatin by weight. The gelatin solution containing mucochloric acid was coated on a transparent cellulose acetate support. A similar gelatin solution to which no hardener had been added was coated on a support, and the two 60

exposed to processing at high temperatures. It was found the latter showed very bad swelling tendencies with the formation of a delicate surface easily susceptible to scratching, whereas 5 the former presented a much more tough and durable surface during processing and resulted in a more satisfactory product when dried.

*Example IV*

10 A hardened filter layer was made as follows: Over a hardened photographic emulsion coated on one side of a transparent support, there was coated a dyed gelatin layer containing mucochloric acid and having the following composition:

|                               | Grams |
|-------------------------------|-------|
| Gelatin solution (5% gelatin) | 100   |
| Congo red dye                 | 2     |
| 20 Mucochloric acid           | .024  |

This coating was permitted to dry and was found to present a tough and durable surface when the film was processed at high temperatures.

*Example V*

25 A hardened anti-halation backing layer was made as follows: A gelatin solution was made up containing gelatin, hardener, and dye in the following amounts:

|                               | Grams |
|-------------------------------|-------|
| Gelatin solution (5% gelatin) | 100   |
| Mucochloric acid              | .12   |
| Anti-halation dye             | 2     |

30 This solution was coated on the back of a cellulose acetate support and permitted to dry.

35 Coatings of emulsions to which the hardening agents have been added were subjected to incubation tests for seven days at 115° F. to determine the extent of fog formation. At the end of this time, the incubation tests showed no more fog than was produced in control samples subjected to a similar incubation test.

40 The amount of hardening agent used, according to my invention, may vary from about 0.1 percent to about 0.5 percent of the weight of the gelatin in the emulsion. The hardening agent may be added to the gelatin used to produce the emulsion at some stage before emulsification, or to the emulsion itself prior to coating. The hardening agents of my invention may also be mixed with gelatin to be used as layers other than emulsion layers on the photographic support, such as backing or anti-halation layers, 45 or inter-layers coated between emulsion layers or between emulsion layers and support. For inter-layers, the amount of aldehyde acid may vary from about 0.1% to about 0.5% of the weight of the gelatin, while for backing and anti-halation layers the amount may vary from about 0.4% to about 3.0% or more.

45 When the hardening agents which I contemplate using are added to certain photographic emulsions, a decrease in sensitivity results. This is apparently due to a lowering of the pH of the emulsion by the acid used as a hardening agent. For this reason in emulsions with a pH of more than 7, it is advisable to use a salt of the acid hardening agent and to adjust the pH of the solution of the acid which is added to the photographic emulsion or gelatin solution. In this way satisfactory hardening is obtained, and in the case of photographic emulsions, the sensitivity is not impaired through the decreased pH produced by the presence of the acids. Sodium

5 or other salts of the halogen-substituted aldehyde acids may be used. These include salts of organic alkalis, such as triethanolamine,  $\beta$ -diethylaminoethyl alcohol, or morpholine, as well as metallic salts.

5 In Fig. 1 of the accompanying drawing, which is an enlarged sectional view of a film made according to my invention, 10 represents a transparent support of glass, cellulose acetate, or other suitable material coated with an emulsion 10 layer 11 consisting of a gelatino-silver halide emulsion hardened with a halogen-substituted aldehyde, such as mucobromic or mucochloric acid.

15 In Fig. 2, which is an enlarged sectional view of a film used in three-color photography, 10 represents a transparent support of cellulose nitrate, cellulose acetate, cellulose acetate propionate, or other suitable material, having emulsion layers 12 and 13 on one side thereof, and emulsion layer 14 20 on the opposite side thereof. Between emulsion layers 12 and 13, there is a hardened gelatin inter-layer 15, and over emulsion layer 14 there is a hardened gelatin filter layer 16.

25 Fig. 3 shows a film having a hardened anti-halation layer 18 coated on the back of support 10, and emulsion layer 17 on the face of the support.

30 It is to be understood that other layers, such as subbing layers and non-curling layers may be added to the photographic element within the scope of my invention.

35 The halogen-substituted aldehyde acids are soluble in various solvents which may be used to incorporate the acid in the gelatin or emulsion. These solvents include water, the alkyl alcohols, and lower esters. Any other suitable solvent which does not adversely affect the gelatin or emulsion may also be used.

40 The examples and compounds included in the above specification are to be taken as illustrative only, since my invention is to be considered as limited only by the scope of the appended claims.

What I claim is:

1. A photographic element comprising a gelatin 45 layer containing as a hardening agent a halogen-substituted aldehyde acid compound.

2. A photographic element comprising a gelatin layer containing as a hardening agent a halogen-substituted aldehyde acid.

3. A photographic element comprising a gelatino-silver halide emulsion layer containing as a hardening agent a halogen-substituted aldehyde acid compound.

4. A photographic element comprising a gelatino-silver halide emulsion layer containing as a hardening agent a halogen-substituted aldehyde acid.

5. A photographic element comprising a gelatino-silver halide emulsion layer containing as a hardening agent mucobromic acid.

6. A photographic element comprising a gelatino-silver halide emulsion layer containing as a hardening agent mucochloric acid.

7. The method of hardening a photographic 65 gelatin, which comprises incorporating therein a halogen-substituted aldehyde acid compound.

8. The method of hardening a photographic gelatin, which comprises incorporating therein a halogen-substituted aldehyde acid.

9. The method of hardening a gelatino-silver halide emulsion which comprises incorporating therein a halogen-substituted aldehyde acid.

10. The method of hardening a gelatino-silver 75

halide emulsion which comprises incorporating therein mucobromic acid.

11. The method of hardening a gelatino-silver halide emulsion which comprises incorporating therein mucochloric acid.

12. The method of producing a hardened gelatino-silver halide emulsion layer which comprises mixing an alcoholic solution of a halogen-substituted aldehyde acid with the emulsion, and 10 coating the mixture on a support.

13. The method of producing a hardened gelatino-silver halide emulsion layer which comprises adding to a gelatino-silver halide emulsion about 15 percent by volume of an alcoholic solution containing about 0.2 percent of the weight of the gelatin in the emulsion of a halogen-substituted

aldehyde acid, and coating the mixture on a transparent support.

14. The method of producing a hardened gelatino-silver halide emulsion layer which comprises adding to a gelatino-silver halide emulsion about 5 percent by volume of an alcoholic solution containing about 0.3 percent of the weight of the gelatin in the emulsion of mucobromic acid, and 5 coating the mixture on a transparent support.

15. The method of producing a hardened gelatino-silver halide emulsion layer which comprises adding to a gelatino-silver halide emulsion about 10 percent by volume of an alcoholic solution containing about 0.5 percent of the weight of the gelatin in the emulsion of mucochloric acid, and 15 coating the mixture on a transparent support.

FRANK L. WHITE.